

## UNITED STATES PATENT OFFICE.

CHRISTINE SIMANEK CUSSEN, OF CHICAGO, ILLINOIS.

## COMPOSITION OF MATTER AND PROCESS FOR PRODUCING THE SAME.

No Drawing.

Application filed April 21, 1924. Serial No. 708,051.

My invention relates to a composition of matter and the process for producing the same, said composition of matter being an alloy preferably resulting from the combination of the following ingredients:

|                                           |           |
|-------------------------------------------|-----------|
| Copper-----                               | 480 parts |
| Nickel-----                               | 144 parts |
| Zinc-----                                 | 160 parts |
| Bronze (copper 16 parts, tin 1 part)----- | 48 parts  |
| 10 and the reaction therewith of          |           |
| Wood charcoal-----                        | 4 parts   |
| White arsenic (arsenic oxide)-----        | 1 part    |

I find that a number of these ingredients may be varied in quantity and still obtain a substance adapted to perform substantially the same functions. From the above proportions I may vary the amount of copper from 480 parts to 704 parts. From the amount of nickel given I may vary the quantity from 144 parts to 288 parts. From the quantity of zinc given I may vary this amount from 160 parts to 224 parts. From the amount of bronze given above I may vary this from 48 parts to 96 parts. I prefer to use bronze made up of 16 parts copper to 1 part tin, but this proportion of copper and tin may be varied through a considerable scope without materially altering the qualities of the resultant material. I prefer to use approximately the quantities of charcoal and arsenic given above in whatever variations of the quantities of the metals which are used. Stating the above quantities in percentages it is apparent that the copper in the alloy may vary from 60.8% to 62.72%; the nickel may vary from 17.2% to 21.88%; the zinc may vary from 17% to 19.12%; the tin may vary from .36% to .45%; while the charcoal used in production of the alloy may vary from .8% to .48%, and the white arsenic may vary from .07% to .12%.

In making up the alloy of my invention, I preferably use a crucible or retort of a size and quality to withstand the required heat and hold the required quantity of metal. I preferably introduce the charcoal in a layer at the bottom of the crucible and then place on the charcoal a layer of nickel in the form generally known as shot nickel. On the nickel, I place a layer of bronze, which is preferably soft sheet bronze and may be scrap or sheet bronze cuttings. On the bronze, I place a layer of copper in the form of ingot copper. The crucible is then placed

in a suitable furnace and heat applied to melt the metals, and after the metals have been melted they are stirred by any convenient means and the temperature thereof raised to a degree between 1500° and 1800° centigrade. Instead of introducing the charcoal in a layer at the bottom of the crucible, it may be added to the molten mass of metals while the same is being stirred but it is preferred to introduce the charcoal in a layer at the bottom of the crucible because of the protection it affords for the crucible, making it possible to use the latter for a larger number of heats.

After the desired degree of heat has been reached, zinc, in the form of block zinc, is stirred into the molten mass before the temperature of the same falls below the melting temperature of zinc; that is to say, while the molten mass is still at a high temperature, the zinc is placed in the molten metal and the latter stirred during the process of adding the zinc. After the zinc has been added, the crucible is removed from the furnace and before the molten mass solidifies, arsenic, in the form of commercial white arsenic or arsenic oxide, is stirred into the molten mass to secure an intimate union for binding of the metals forming the alloy. When carbon is added to the molten mass, it should be done before the zinc is added and while the molten mass is being stirred. Then the zinc is stirred into the molten mass and finally the white arsenic is stirred into the molten mass. If desired, the zinc may be previously melted and the white arsenic mixed therewith and then the mixture of the molten zinc and white arsenic stirred into the bath of the crucible.

The resultant mixture is then cast into ingots or any other desired form and is then ready to be recast into various desired articles. The resultant metal alloy which is thus produced contains copper, tin, nickel and zinc but substantially no charcoal nor arsenic since the carbon and the arsenic are for the purpose of acting as a flux to remove impurities from the metals, copper, tin, nickel and zinc, and thereby permit the desired union or binding of the metals while they are in the molten state. This flux, by removing the impurities from the metals specified, forms a slag which rises to the top of the melt where it may be conveniently removed. If more charcoal and arsenic are used than necessary to remove impurities

from the bath, the quantity of carbon and arsenic which will find its way into the alloy would be very small or a mere trace of each.

5 The metal may be cast directly into such articles as it is to be finally used in without being cast in ingots when so desired.

The object of this invention is the production of a new alloy or metal which retains its polish or lustre after it is once given such finishes, and a metal which will resist corrosion. This alloy or metal is very desirable for builder's hardware, golf irons, surgical instruments, and all other tools or instruments where a reasonable amount of strength is required, and which are subject to being easily and quickly corroded. It is also very suitable for use in forming bearings or where friction alleviating means is desirable. It is also an excellent alloy for valves, valve seats, etc. which are subject to agencies which tend to promote corrosion.

This metal retains a finish given it, and has the advantage over plated goods in that 25 there is no plate to wear off or to become loosened from the article, since it is of the same composition throughout. This alloy or metal is stronger and tougher than brass, and is, therefore, adapted for a greater range 30 of uses than is brass or copper.

While I have illustrated and described the preferred amounts of ingredients making up the alloy of my invention, and the preferred method of making such alloy or metal, I do 35 not desire to be limited to the exact details set forth, but desire to avail myself of such variations and changes as fall within the scope of the appended claims.

I claim:

40 1. The process of forming an alloy consisting of heating together charcoal, nickel, bronze and copper to a temperature considerably higher than the melting temperature of any of said metals; agitating the 45 mixture during said heating; adding zinc to the mixture while the latter is being agitated and heat applied thereto; discontinuing the application of heat; and adding white arsenic to the mixture while the latter is still in the molten state, agitating the 50 mixture while adding the white arsenic.

2. The process of forming an alloy consisting of heating together charcoal, nickel, bronze and copper to a temperature considerably higher than the melting point of 55 any of said metals; stirring the mixture after said metals have been melted; stirring the zinc into the mixture after said high temperature has been reached and before the 60 application of heat is discontinued from the mixture; and stirring white arsenic into the mixture after the application of heat has been discontinued and while the mixture is still in a molten state.

65 3. The process of forming an alloy con-

sisting of heating together charcoal, nickel, bronze and copper to a temperature considerably higher than the melting temperature of any of said metals; stirring the mixture after said metals have been melted; 70 stirring zinc into the mixture after the latter has been brought to a high temperature, and stirring white arsenic into the mixture before the latter has reached a solid state.

4. The process of forming an alloy consisting of placing together in a container layers of carbon, nickel, bronze and copper in the order named; heating the ingredients to approximately 1800° centigrade, more or less; stirring the ingredients after the metals 80 have been melted; stirring zinc into the molten mixture after said metals have been brought to said high temperature; and discontinuing the application of heat to the mixture then stirring white arsenic into the 85 mixture before the latter has been cooled to a solid state.

5. The process of forming an alloy of nickel, copper, tin and zinc, which consists in heating together charcoal, a compound 90 of arsenic, nickel, bronze, and copper to a temperature sufficient to melt said metals, stirring the mixture while in the molten state and then adding zinc.

6. The process of forming an alloy of 95 nickel, copper, tin and zinc, which consists in mixing said metals with carbon while said metals are in the molten state and also stirring white arsenic into the mixture while said metals are still in the molten state. 100

7. The process of forming an alloy of nickel, copper, tin and zinc which consists in first mixing nickel, bronze and copper with carbon while said nickel, bronze and copper are in a molten state, then stirring zinc into the mixture, and afterward stirring white arsenic into the mixture comprising nickel, copper, tin and zinc, and while the latter are still in the molten state. 105

8. The process of forming an alloy of 110 nickel, copper, tin and zinc, which consists in placing in a container layers of carbon, nickel, bronze, and copper; heating the container ingredients to effect the melting of said nickel, bronze and copper, stirring zinc 115 into the molten mixture, and then stirring white arsenic into the mixture comprising nickel, tin, copper and zinc.

9. The process of forming an alloy of 115 nickel, copper, tin and zinc, which consists in heating nickel, bronze and copper with carbon to a temperature higher than the melting point of either nickel, bronze or copper; stirring the mixture after the said nickel, bronze and copper have been melted; stirring zinc into the mixture of nickel, tin and copper; and stirring white arsenic into the mixture comprising nickel, tin, copper and zinc. 125

10. The process of forming an alloy of 130

nickel, copper, tin and zinc, which consists in heating nickel, bronze and copper in close proximity to carbon until the said nickel, bronze and copper are melted, then stirring the ingredients while continuing the heating and adding zinc to the molten mixture during such stirring; and then discontinuing the application of heat to the mixture and stirring white arsenic into the mixture before

10 it reaches a solid state.

11. The process of forming an alloy non-corrodible under ordinary natural atmospheric conditions, consisting of heating together nickel, bronze and copper to a temperature higher than the melting point of any one of the said metals, adding carbon to the molten mass while the same is being stirred, stirring zinc into the molten mass before the temperature of the same falls

15 below the melting temperature of zinc and stirring white arsenic into said alloy before the same solidifies.

12. The process of forming an alloy non-

corrodible under ordinary natural atmospheric conditions, consisting of heating together nickel, tin and copper to a temperature higher than the melting point of any one of the said metals, adding carbon to the molten mass while the same is being stirred, stirring zinc into said molten mass before the temperature of the same falls below the melting temperature of zinc and stirring an arsenic compound into the same.

13. The process of forming an alloy non-corrodible under ordinary natural atmospheric conditions, consisting of heating together nickel, tin and copper to a temperature higher than the melting point of said metals, adding carbon to the molten mass while the same is being stirred, and stirring 40 a mixture of molten zinc and white arsenic into said molten mass.

In testimony whereof I have signed my name to this specification on this 18th day of April, A. D. 1924.

CHRISTINE SIMANEK CUSSEN.